

Jan. 3, 1928.

1,655,371

H. O. KEAY

METHOD OR PROCESS OF CEMENTING PULP STONES

Filed May 19, 1924

A PHENOLIC FORMALDEHYDE RESIN  
IN FURFURAL



FIG.1

A PHENOLIC FORMALDEHYDE RESIN  
IN FURFURAL & SAND



FIG.2

INVENTOR  
HERBERT O. KEAY

BY *Fetherstonhaugh & Co*  
ATTORNEYS

## UNITED STATES PATENT OFFICE.

HERBERT O. KEAY, OF GRAND MERE, QUEBEC, CANADA, ASSIGNOR TO LAURENTIDE COMPANY, LIMITED, OF GRAND MERE, QUEBEC, CANADA.

## METHOD OR PROCESS OF CEMENTING PULP STONES.

Application filed May 19, 1924. Serial No. 714,499.

This invention relates to a method or process of cementing or binding together two pulp stones of moderate thickness with an abrasive cement in order to form a comparatively large stone of suitable thickness for grinding pulp wood in magazine grinders.

In the production of pulp stones from sand stone quarries, considerable difficulty is experienced in obtaining sufficient masses of clear sand-stone material, free from defects, from which to turn out finished stones suitable for grinding logs, such stones having, say, a finished diameter of sixty-two inches with a face width of fifty-four inches.

15 It is estimated that from twelve to fifteen stones of the same diameter, but of half the face width, could be turned out for every single stone of the larger face width of fifty-four inches.

20 In order to produce a grinding stone by cementing or binding together two or more stones of smaller size, it is obvious that the binding material must possess certain very important qualities. It must, for instance, be essentially insoluble in hot water, must be a strong adhesive, must not crumble away in service, thus leaving a crack or opening or, in other words, it must contain an abrasive aggregate to do its part in grinding 25 evenly. The binding material must, further, be sufficiently hard to re-inforce the edges of the stone so that crushing off of the stone will not take place when the dressing burr is forced across the face of the stone. This 30 binding material must, further, be sufficiently porous so that glazing will not take place at the grinding surface of the cement.

I have found that the above-mentioned qualities are obtained by using a resin dissolved in an organic solvent as a binder for an abrasive aggregate. For instance, I use a phenolic formaldehyde resin dissolved in furfural solvent for a binder, and sand as an abrasive aggregate, and this binder, when 40 applied in the manner hereinafter described, produces a grinding stone possessing all the necessary requirements. The phenolic formaldehyde resin, is preferably such as set forth in British Patent No. 9291 of 1914 to 45 Laurence Vincent Redman. Resins of this character are formed by incorporating hexa-

methylenetetramine with a phenol and heating the mixture, the excess of either reagent being removed or left in the compound as desired. Resins of this character may be 55 manufactured by mixing the ingredients in suitable proportions to form a product which can be converted into an insoluble infusible chemically inert substance. The proportions are as follows: one and one half phenol 60 groups to one methylene group, or at least, nine molecules of phenol to one molecule of hexamethylenetetramine.

In the accompanying drawings, Figure 1 illustrates two stones with their adjacent 65 surfaces prepared for cementing them together, and Figure 2 is a part sectional elevation of two stones cemented together according to my invention.

In carrying out the process of cementing 70 the stones together I first thoroughly coat the surface by any suitable means, such as a stiff brush, with a solution of a phenolic formaldehyde resin dissolved in furfural solvent. With ordinary sand-stones used 75 for pulp grinding no further preliminary treatment of the surface is required, but if the sand-stone is exceptionally porous, I find it preferable to bake the stones after the preliminary coating has been applied. This 80 baking treatment may be carried on for twenty-four to forty-eight hours at a temperature of approximately 130° C. I then coat the surfaces to be cemented together with an abrasive cement which is made by 85 mixing a fine clean sand with a suitable quantity of a phenolic formaldehyde resin and to this mixture is added a suitable amount of furfural solvent, the whole mass then being thoroughly mixed and kneaded 90 until all the grains of sand are thoroughly moistened by the dissolved resin. This abrasive cement is spread evenly to a depth of about one-sixteenth of an inch over one, or both, of the stone surfaces which have been 95 previously coated, as above described. The two surfaces are then pressed together firmly and clamped, for greater security in handling, while the cement is still plastic. The clamped stones are then placed in an oven 100 and kept at a temperature of 130° to 150° C. for approximately two days. The tem-

perature is then raised to about 170° C. for approximately twenty-four hours longer. After this, the cemented stone is removed from the oven, unclamped, and allowed to cool slowly. It is important that no considerable delay should occur in the process after the resin has been mixed with the solvent as polymerization of the resin begins, to some degree, under ordinary atmospheric conditions. A phenolic formaldehyde resin or any similar artificial resin capable of solution by an organic solvent may be used in making this abrasive cement. As the abrasive cement constitutes the subject matter of another patent application filed by me it need not be specifically described in this application which is directed only to the process of cementing the stones together.

Having thus described my invention, what I claim is:—

1. A process of cementing two or more stones together which consists in, first, coating the surfaces to be cemented with a solution of a phenolic formaldehyde resin dissolved in an organic solvent, and then coating the prepared surfaces with an abrasive cement, clamping the stones together, then heating the stones for approximately forty-eight hours to a temperature of 130° to 150° C. and then increasing the heat to approximately 170° C. for a further period of twenty-four hours, then removing the stones and allowing same to cool.
2. A process of cementing two or more sand-stones together to form a pulp grinding stone which consists, in first, coating the surfaces to be cemented with a binder consisting of a phenolic formaldehyde resin dissolved in furfural solvent and then coating the treated surfaces with an abrasive cement consisting of fine sand mixed with phenolic formaldehyde resin and furfural solvent, then baking the cemented stones for approximately forty-eight hours at a temperature of 130° to 150° C. and then increasing the temperature to 170° C. for a further period of twenty-four hours.
3. A pulp grinding stone consisting of several parts having their adjacent surfaces coated with a solution of a phenolic formaldehyde resin dissolved in an organic solvent and united by a cement containing sand as an abrasive aggregate, said cement having the grinding qualities of the grinding stone.
4. A pulp grinding stone consisting of several parts having their adjacent surfaces coated with a solution of a phenolic formaldehyde resin dissolved in an organic solvent and united by a cement consisting of fine sand mixed with a phenolic formaldehyde resin and furfural.
5. A pulp grinding stone consisting of several parts having their adjacent surfaces coated with a solution of a resin dissolved in an organic solvent and united by a cement

containing sand, a resin and an organic solvent.

6. The process of cementing two or more stones together which consists in first, coating the surfaces to be cemented with a binder consisting of a resin dissolved in an organic solvent, then coating the so treated surfaces with an abrasive cement consisting of a mixture of sand, a resin, and an organic solvent and then baking the cemented stones.

7. The process of cementing two or more stones together which consists in first, coating the surfaces to be cemented with a binder consisting of a resin dissolved in an organic solvent, then coating the so treated surfaces with an abrasive cement consisting of a mixture of sand, a resin, and an organic solvent, then baking the cemented stones at a relatively high temperature and then subjecting the so baked stones to a further heat treatment at a higher temperature.

8. The process of cementing two or more stones together which consists in first, coating the surfaces to be cemented with a phenolic formaldehyde resin dissolved in an organic solvent, then coating the so treated surfaces with an abrasive cement consisting of a mixture of sand, a phenolic formaldehyde resin and an organic solvent, and then baking the cemented stones.

9. The process of cementing two or more stones together which consists in first, coating the surfaces to be cemented with a phenolic formaldehyde resin dissolved in furfural, then coating the so treated surfaces with an abrasive cement consisting of a mixture of sand, a phenolic formaldehyde resin and furfural, and then baking the cemented stones.

10. The process of cementing two or more stones together which consists in first, coating the surfaces to be cemented with a phenolic formaldehyde resin dissolved in furfural, then coating the so treated surfaces with an abrasive cement consisting of a mixture of sand, a phenolic formaldehyde resin and furfural, then baking the cemented stones at a relatively high temperature and then subjecting the so baked stones to a further heat treatment at a higher temperature.

11. A pulp grinding stone consisting of several parts having their adjacent surfaces cemented together with an abrasive cement comprising sand as an abrasive element, said sand being mixed with a phenolic formaldehyde resin and furfural, the cement aggregate having the grinding qualities of the stone which is united thereby.

12. A pulp grinding stone consisting of several parts of sand stone having their adjacent surfaces cemented together with an abrasive cement comprising sand as an abrasive element, said sand being mixed with a phenolic formaldehyde resin and fur-

fural, the cement aggregate having the grinding qualities of the stone which is united thereby.

13. A pulp grinding stone consisting of several parts of sand stone having their adjacent surfaces coated with a solution of a phenolic formaldehyde resin dissolved in an organic solvent and united by a cement

consisting of fine sand mixed with a phenolic formaldehyde resin and furfural, said 10 cement aggregate having the grinding qualities of the sand stone itself.

In witness whereof, I have hereunto set my hand.

HERBERT O. KEAY.